

# UNITED STATES PATENT OFFICE.

ANDREW O'NEILL, OF NEW HAVEN, CONNECTICUT.

## ELECTROPLATED YELLOW-METAL.

SPECIFICATION forming part of Letters Patent No. 257,605, dated May 9, 1882.

Application filed July 29, 1879.

*To all whom it may concern:*

Be it known that I, ANDREW O'NEILL, a citizen of the United States, residing at New Haven, in the State of Connecticut, have invented a new and useful Improvement in Electroplated Yellow-Metal, of which the following is a specification.

In my specification forming part of Letters Patent No. 179,462, dated July 4, 1876, I describe and claim a "machine-planished, nickel-plated, polished, and enameled sheet of copper, brass, or yellow-metal" as a new article of manufacture, the process therein set forth having reference more particularly to the production of electro-nickelated copper. I have since discovered that ordinary pack-rolled yellow-metal furnishes a better product without being "machine-planished"—that is to say, without being "cold-rolled," owing to the hardening effect of this operation, which unfitts cold-rolled yellow-metal for general use, while the smoothness of this metal as it comes from the pack-rolls renders cold-rolling unnecessary preliminary to electroplating. I have discovered, moreover, that at a trifling expense compared with the advantages which result copper could be evenly electro-deposited on the backs of nickel-plated sheets of yellow-metal, or on one side of a sheet, the other side of which is subsequently electro-nickled, and have so combined the three metals, thereby producing for the first time in the art of manufacturing plated sheet metals (so far as I am informed) an electro-laminated sheet composed of three different metals, while the article of this description to which I propose confining my present invention, composed of a sheet of yellow-metal electroplated with nickel on one side and with copper on its other side, is a cheap and, in many respects, superior substitute for nickel-plated copper, and an article never before known or used.

The adaptation of electro-nickelated and coppered yellow-metal for particular uses at a given weight or cost by the variation of the relative thicknesses of the respective laminæ can be most readily effected and is an element of superiority. For example, for bathtubs and the like, where the nickel surface alone is exposed to wear, a much heavier plating of nickel can be furnished in sheets of a given cost than in nickelated copper sheets, while

the stiffness of the yellow-metal, as compared with copper, renders it superior to solid copper for such uses, and even a light electro-deposit of copper covering its back amply protects it against corrosion.

In producing my said composite sheet of yellow-metal, nickel, and copper I prefer to proceed as follows: Ordinary commercial sheet yellow-metal (pack-rolled) is simply scoured and pickled, or otherwise thoroughly cleansed, so as to prepare both sides to receive an electro-deposit. The sheets are then clamped together in pairs, back to back, by means of edge-clamps, which may be of wire, and the pairs of sheets are suspended between suitable anodes in a nickel-plating bath, and connected with the negative pole of a powerful dynamo-electric machine in customary manner. When the faces of the sheets of yellow-metal have received a nickel-plating of the desired thickness the pairs of sheets are removed from the nickel-bath, unclamped and raised, and the sheets are then reunited in pairs and immersed between copper anodes in a copper bath to electroplate their backs, the respective sheets at each operation forming effective resists for each other without other means, owing to the described relation of the parts in the plating-baths. The extreme edges of the sheets punctured for clamping, and acted on more or less by the plating-currents in both baths, must subsequently be trimmed off; but this "waste" in large operations is more than compensated for by the economy in time and labor as compared with preparing, applying, and removing ordinary resists. The latter may, however, be used in carrying out this invention, the whole of one side of each sheet being reserved at the first plating operation and the previously plated sides at the succeeding plating operation.

The ordinary baths are used for plating, the double sulphate of nickel and ammonia for the nickel and the sulphate of copper for the copper being preferred; but baths of the cyanides of these metals will also answer; and in place of nickel-plating, silver or other noble metal plating may be used; but this I find is in no respect better than nickel-plating, while it is inferior in durability as well as in cheapness.

If a "soft-planished" product, adapted to be

spun or stamped, is desired, the composite sheet, after it is taken from the last plating-bath and dried, is simply buffed and lacquered in the manner described in my aforesaid specification, forming part of Letters Patent No. 179,462, without cold-rolling; but if the composite sheet be intended to be worked up from the sheet by cutting and bending simply, as in the manufacture of culinary vessels, wash-boilers, bath-tubs, and the like, and for ship-sheathing, it is subjected to cold-rolling, which compacts and toughens the electro-deposits before said finishing operations.

The composite sheet is eminently adapted for use in the manufacture of culinary utensils, liquid-measures, wash-boilers, and the like, as the nickelized surface is durable and inoxidizable, while the copper side for the exterior is very much less liable to tarnish than naked yellow-metal, with its large percentage of baser metal, (zinc,) and the stiffness of the yellow-metal base serves with obvious advantage to prevent indentation.

Finished in either of the ways above described the composite sheet works up in the various operations of sheet-metal working—such as double seaming and grooving—as well as ordinary sheet yellow-metal or copper, and soft-

planished, as above set forth, it may be stamped or spun with repeated annealings, if necessary, without injury to the base or either plating, and without impairing the union between the laminæ, while it may be made at a cost less than that of ordinary bright sheet-copper or tinned copper, used for analogous purposes. 35

I do not claim herein the within-described method of reserving the surfaces of metallic sheets in electroplating-baths by means of similar sheets undergoing the same process, nor an electro-laminated sheet composed of 40 three different metals, broadly considered, but hereby reserve the right to claim the same in a future application or applications for Letters Patent.

I claim as my invention and desire to secure 45 by Letters Patent—

As a new article of manufacture, the within-described composite sheet metal, consisting of sheet yellow-metal electroplated on one side with nickel and on its other side with copper, 50 substantially as specified, for the purposes set forth.

ANDREW O'NEILL.

Witnesses:

R. D. WILLIAMS,  
GEO. H. PISTEL.